

## UNITED STATES PATENT OFFICE

2,043,541

## PROCESS OF FINISHING WOOD

Hugh Jamieson, Stamford, Conn.

No Drawing. Application March 2, 1936,  
Serial No. 66,732

7 Claims. (Cl. 91—70)

My invention relates to my application Serial No. 47,274, filed October 29, 1935, of which this is a continuation in part and particularly pertains to that class of materials which are designed to 5 protect the wood, as well as impart a pleasing aspect for the wood when finished.

It is well known that when wooden golf clubs are in use they are frequently wet and dry—wet and dry, moreover they are not only struck by the 10 impact of the ball but they also strike against the irons in the bag. This tends to crack or check the varnish, moisture frequently gets into the club and sometimes lifts the varnish off causing an unsightly appearance of the club and even- 15 tually destroying its utility. This is due to the fact that the finish is on the surface of the wood.

Tennis racquets are extremely susceptible to the weather and in fact cannot be safely used in damp weather.

20 The best finish when applied to table tops is easily damaged by the application of heat from hot plates or dishes or by spilling alcohol or acids on them so that the top must be refinished.

On boats, especially on salt water, even the 25 finest finishes on deck, spars, blocks, etc., deteriorate very rapidly. When the hulls are mahogany, a roughness soon appears which holds the boat back in the water and consequently retards the speed.

30 My invention has for its object to provide a finish which will entirely obviate all of the foregoing objections which instead of finishing the surface of the wood will actually impregnate it, so that there is no surface finish to check, peel or 35 crack.

A further object is to produce a finish which is susceptible of a high polish if that is desired or will furnish a dull or mat finish for the wood.

40 A further object is to provide a finish which will not roughen up when subjected to the action of salt water.

A further object is to produce a finish which will not be injured by heat, alcohol or acids.

45 My process consists essentially of the following steps:—I prepare a finish as follows: 33 1/3% of linseed oil which has been brought up to a temperature of 212 degrees F., 33 1/3% of a composition formed of 2 oz. kauri resin, 4 1/2 ounces raw China wood oil, 50 1 1/2 ounces turpentine, 2 1/2 ounces "Varnolene," 2 1/2 cc. cobalt drier, 17% of pure beeswax, and 16 1/3% of wood filler, heating the wax, oil and 55 filler to approximately 212 degrees F., adding the composition, then heating until the mass is a liquid, applying the liquid to the wood, cooling the impregnated wood rapidly, and then buffing the cooled wood.

without departing from the spirit of my invention as hereinafter claimed.

I first heat the wax, oil and filler to approximately 212 degrees F. then add the composition compounded of the ingredients described in the preceding paragraph. When the wood to be finished is a table top, the finish is heated to approximately 212 degrees F. and is applied while hot. The wood is then cooled rapidly. This may be done in any approved manner. When 10 the wood is cooled the surface can be buffed to obtain the desired gloss.

For small articles such as golf clubs, tennis racquets, etc., I find it better to immerse them a number of times in the liquid. For example, I 15 have found that very desirable results are obtained by having the liquid at 212 degrees F. for the first dip; 25 degrees F. less for the second dip and approximately 100 degrees F. for the third dip. For wood to be used on boats, I build a tank 20 of sufficient size to permit the complete board or boards to be placed therein so that the entire surface will be immersed in the hot liquid. When the boards are removed from the tank and cooled they may be applied to the hull, deck or other 25 location and then buffed until the desired surface polish is secured. Although I have described with some degree of particularity the manner of using my finish, the description is only for the purpose of supplying a concrete embodiment of 30 my process and I do not desire to be understood as limiting myself to the precise steps set forth except as such limitations may be found in the hereinafter contained claims.

Having described my invention what I regard 35 as new and desire to secure by Letters Patent is—

1. A process of finishing wood, which consists of the following steps: forming a finish of boiled linseed oil, 33 1/3% of a composition formed of 2 oz. kauri resin, 4 1/2 ounces raw China wood oil, 40 1 1/2 ounces turpentine, 2 1/2 ounces "Varnolene," 2 1/2 cc. cobalt drier, 17% of pure beeswax, and 16 1/3% of wood filler, heating the wax, oil and 45 filler to approximately 212 degrees F., adding the composition, then heating until the mass is a liquid, applying the liquid to the wood, cooling the impregnated wood rapidly, and then buffing the cooled wood.

2. A process of finishing wood which consists 50 of the following steps: providing a finish formed of 33 1/3% of boiled linseed oil, 33 1/3% of a composition formed of 2 oz. kauri resin, 4 1/2 ounces raw China wood oil, 1 1/2 ounces turpentine, 2 1/2 "Varnolene," 2 1/2 cc. cobalt drier, 17% of pure beeswax, 16 1/3% of wood filler, heating the wax, 55

oil and filler to approximately 212 degrees F., adding the composition, then heating until the mass is a liquid, immersing the wood in the liquid, cooling the impregnated wood, and then buffing the cooled wood.

5. 3. The process of treating wood which comprises immersing wood to be finished in a heated liquid formed of the following ingredients, boiled linseed oil, 33 1/3% of a composition formed of 2 oz. kauri resin, 4 1/2 ounces raw China wood oil, 1 1/2 ounces turpentine, 2 1/2 ounces "Varnolene", 2 1/2 cc. cobalt drier, pure beeswax, and wood filler, cooling the impregnated wood, and then buffing the cooled wood.

10. 4. A process of finishing wood which consists of the following steps: forming a finish of 33 1/3% of boiled linseed oil, 33 1/3% of a composition formed of 2 oz. kauri resin, 4 1/2 ounces raw China wood oil, 1 1/2 ounces turpentine, 2 1/2 ounces "Varnolene", 2 1/2 cc. cobalt drier, 17% of pure beeswax, and 16 2/3% of wood filler, heating the wax, oil and filler to approximately 212 degrees F., adding the composition, then heating until the mass is a liquid, and immersing the wood to be finished in the liquid.

15. 5. A process of finishing wood which consists of the following steps: forming a finish of 33 1/3% of boiled linseed oil, 33 1/3% of a composition of 2 oz. kauri resin, 4 1/2 ounces raw China wood oil,

1 1/2 ounces turpentine, 2 1/2 ounces "Varnolene", 2 1/2 cc. cobalt drier, 17% of pure beeswax, and 16 2/3% of wood filler, heating the wax, oil and filler to approximately 212 degrees F., adding the composition, then heating until the mass is 5 a liquid, immersing the wood to be finished in the liquid while heated to approximately 212 degrees F., redipping the wood in the liquid when it is cooled to approximately 187 degrees F., then redipping the wood with the liquid cooled to 10 approximately 100 degrees F., then cooling the impregnated wood, and then buffing the cooled wood.

15. 6. A finish for wood consisting of 1/3 of boiled linseed oil, 1/3 of a composition formed of 2 oz. 15 kauri resin, 4 1/2 ounces raw China wood oil, 1 1/2 ounces turpentine, 2 1/2 ounces "Varnolene", 2 1/2 cc. cobalt drier, 1/6 of pure beeswax and 1/6 of wood 20 filler, formed by first heating the wax, oil, and filler, and then adding the composition.

25. 7. A finish for wood comprising a liquid formed of boiled linseed oil, a composition formed of kauri resin, raw China wood oil, turpentine, "Varnolene", cobalt drier, pure beeswax, and wood filler, the wax, oil and filler to be heated to approximately 212 degrees F. before adding the composition.

HUGH JAMIESON.